

1

2,939,843

## ANTIWEELD AND ANTIWEAR LUBRICATING OIL COMPOSITION

John N. Bowden and Paul R. Chapman, Crystal Lake, Ill., assignors to The Pure Oil Company, Chicago, Ill., a corporation of Ohio

No Drawing. Filed Aug. 23, 1956, Ser. No. 605,697

4 Claims. (Cl. 252—37.2)

This invention relates to lubricating oils and more particularly to lubricating oils capable of withstanding high loads.

It is common practice to incorporate into mineral lubricating oils intended for lubricating automotive gears and other mechanical parts subject to extreme pressures, additives which are capable of enhancing the load-carrying properties of the oil. Among the additives commonly used for this purpose, particularly in break-in oils or oils intended for lubricating "green gears," are lead naphthenate and free sulfur. Lead naphthenate and free sulfur, however, have the drawback of causing high wear under low speed-high torque conditions. In other words, although the combination of lead naphthenate and sulfur impart satisfactory anti-weld characteristics to the oil, it is not a satisfactory E.P. additive combination under the varied conditions encountered in service.

We have discovered that if a small amount of a haloalkyl phosphite is incorporated into the oil containing sulfur, with or without lead naphthenate, the anti-wear properties of the oil are materially improved while the anti-weld properties of the oil remain at a high level.

An object of our invention is to provide a new lubricating oil composition. Another object of our invention is to provide an extreme pressure gear oil which is satisfactory both under high speed-low torque and low speed-high torque operating conditions. A still further object of the invention is to provide a lubricant having good anti-wear and anti-weld properties. Other objects of the invention will manifest themselves from the following description.

2

halogenated phosphite ester used, but in general should not exceed about five times by weight the amount of free sulfur present in the oil. For example, if the oil contains 0.2% of free sulfur, the phosphite should not exceed about 1% by weight of the oil composition.

In preparing lubricating oils in accordance with our invention, a mineral lubricating oil of desired viscosity and other properties is blended with about 0.5 to 5% of lead naphthenate and 0.05 to 1% of sulfur. An oil of this composition has excellent load-carrying characteristics as indicated by the four-ball weld test, but has a poor wear-preventive characteristics as demonstrated by the four-ball, 5-minute wear test. The four-ball test for determining load-carrying and wear properties is briefly described on pages 13 and 14 of "The Performance of Lubricating Oils," by Zuideman, published in 1952 by Reinhold Publishing Corp., New York. To improve the wear characteristics of this oil, a small amount of a halogenated phosphite ester of the order of 0.1 to 5% by weight is incorporated in the oil. As examples of halogenated phosphite esters which may be used are tri(chloroethyl) phosphite, chlorooctyl dihydrogen phosphite, di(chlorooctyl) hydrogen phosphite, tri(bromopropyl) phosphite, tri(bromohexyl) phosphite, di(bromoheptyl) hydrogen phosphite, tri(chlorooctyl) phosphite, tri(chlorobutyl) phosphite, tri(chloroamyl) phosphite, and tri(chlorolauryl) phosphite. The partial esters may be so strongly acidic as to be corrosive to the metal, in which case either the quantity of the partial ester in the blend can be reduced, or the blend can be treated with basic oxides or hydroxides, such as those of calcium, barium, zinc, lead, etc., or with basic nitrogen compounds, such as ammonia and amines, in order to eliminate corrosivity. Haloalkyl phosphites containing from 1 to 30 carbon atoms in the alkyl radicals are satisfactory, as long as the compounds are substantially non-volatile under service conditions and are sufficiently soluble in the oil so that they remain in solution and will not precipitate out during storage or in service.

40 In order to illustrate the invention, a number of blends were prepared by mixing with mineral lubricating oil, lead naphthenate, sulfur and several different phosphorus compounds until a homogeneous solution was obtained. Blends were tested on the four-ball machine. The results of the tests are given in the following table.

Table I

| Composition, parts by weight                                        | Blend Number |         |       |         |       |         |       |         |
|---------------------------------------------------------------------|--------------|---------|-------|---------|-------|---------|-------|---------|
|                                                                     | 1            | 2       | 3     | 4       | 5     | 6       | 7     | 8       |
| Lead naphthenate                                                    | 4.0          | 4.0     | 4.00  | 4.0     | 4.00  | 4.0     | 4.0   | 4.0     |
| Sulfur                                                              | 0.1          | 0.25    |       | 0.2     | 0.08  | 0.1     | 0.1   | 0.1     |
| Tri(chloroethyl) phosphite                                          |              |         | 1.0   | 1.00    |       |         |       |         |
| Extract-P <sub>4</sub> S <sub>6</sub> reaction product              |              |         |       |         |       |         | 1.0   |         |
| Diethyl dithiophosphoric acid                                       |              |         |       |         |       | 1.0     |       |         |
| Zinc salt of extract-P <sub>4</sub> S <sub>6</sub> reaction product |              |         |       |         |       |         |       |         |
| Mineral oil                                                         | 96.0         | 95.9    | 95.75 | 94.8    | 94.92 | 94.9    | 94.9  | 94.9    |
| 4-Ball E.P. Machine 5 minute wear, -20 kg. load                     |              |         |       |         |       |         |       |         |
| Scar diameter (mm.)                                                 | 0.389        | 0.306   | 0.412 | 0.209   | 0.305 | 0.419   | 0.386 | 0.389   |
| Weld point (kg.)                                                    | 170-180      | 530-540 | >810  | 500-580 | <400  | 460-480 | <420  | 460-480 |

In carrying out our invention it is important to adjust the quantities of sulfur and haloalkyl phosphite so that the phosphite does not markedly detract from the anti-weld properties of the sulfur and lead naphthenate. We have found that if the proportion of phosphite to sulfur is too large, although the anti-wear properties of the oil are improved, the anti-weld properties are reduced below a satisfactory level so that the oil will not operate satisfactorily as a break-in oil for "green gears." The amount of phosphite will depend to some extent on the particular

From an examination of the table it will be seen that lead naphthenate alone imparts relatively poor load-carrying and wear-resistant properties to the oil as measured by the weld point and scar diameter. Incorporation of 0.1% of sulfur materially increases the load-carrying properties as demonstrated by the increase in the weld point, but the wear-resistance of the oil is adversely affected by the incorporation of the sulfur. This tendency to detract from wear and to improve load-carrying properties is further augmented by addition of

more sulfur as shown by Blend No. 3. Upon addition of 1% of tri(chloroethyl) phosphite to a blend containing 4% of lead naphthenate and 0.2% of sulfur, the anti-wear property of the oil was materially improved while the load-carrying properties of the oil remained at a high level. Blend No. 5 demonstrates that the ratio of sulfur to tri(chloroethyl) phosphite is too low to obtain satisfactory load-carrying characteristics.

Blends 6, 7 and 8 demonstrate that other phosphorus-containing additives were not effective in improving the wear characteristics of the oil while at the same time they detracted from the load-carrying characteristics of the oil.

The blends included in the table were made from mineral oil having the following characteristics:

|                |      |
|----------------|------|
| Vis./210° F.   | 85.3 |
| Vis./130° F.   | 441  |
| Vis./100° F.   | 1148 |
| V.I.           | 74   |
| Pour pt., ° F. | +10  |
| API gravity    | 23.1 |
| Percent S      | 1.13 |

The extract- $P_2S_5$  reaction product used in some of the blends was made by reacting at about 220°-230° F., for four hours, 10 parts by weight of phosphorus pentasulfide and 1 part of aromatic extract obtained from the extraction of a neutral fraction with phenol.

The zinc salt of the extract- $P_2S_5$  reaction product was made by neutralizing the extract- $P_2S_5$  reaction product above-described with zinc oxide at a temperature of about 250° F. The extract used in making this product had the following characteristics:

|                      |       |       |
|----------------------|-------|-------|
| Viscosity at 100° F. | SUS   | 165.5 |
| Gravity              | ° API | 17.3  |
| Flash point          | ° F.  | 375   |

Fire point \_\_\_\_\_ ° F. 430  
 Acid number \_\_\_\_\_ 3.8  
 Sulfur \_\_\_\_\_ percent 2.03

5 By blending together a haloalkyl phosphite with lead naphthenate and sulfur into a lubricating oil, a product is made which is effective both as a break-in oil for automotive gears and as a lubricant for use under ordinary service so that the break-in oil does not have to be changed after the gears are broken in but can be left in the transmission without fear of causing excess wear of the gear teeth.

10 We claim as our invention:

1. A lubricating oil consisting essentially of a mineral oil of lubricating oil grade, a minor amount of lead naphthenate, 0.05-1.0 wt. percent sulfur, 0.25-5.0 wt. percent of a  $C_1-C_{10}$  haloalkyl phosphite, with a ratio of phosphite to sulfur in the range of 2 to 5:1, said phosphite enhancing the antiwear properties of the oil without detracting substantially from the anti-weld properties thereof.

15 2. A lubricating oil in accordance with claim 1 in which the phosphite is a tri(chloroalkyl) phosphite.

20 3. A lubricating oil in accordance with claim 2 in which the phosphite is tri(chloroethyl) phosphite.

25 4. A lubricating oil in accordance with claim 1 in which all of the haloalkyl phosphite present is in solution in the oil.

#### References Cited in the file of this patent

#### UNITED STATES PATENTS

|           |                  |               |
|-----------|------------------|---------------|
| 2,169,185 | Shoemaker et al. | Aug. 8, 1939  |
| 2,176,426 | Kaufman et al.   | Oct. 17, 1939 |
| 2,298,636 | Prutton          | Oct. 13, 1942 |
| 2,722,517 | Smith et al.     | Nov. 1, 1955  |